

# UNITED STATES PATENT OFFICE.

FOSTER MILLIKEN, OF LAWRENCE, NEW YORK, ASSIGNOR TO FOSTER MILLIKEN, S. FULLERTON WEAVER AND JAMES M. REPLIER, AS TRUSTEES.

## ALLOY.

1,393,388.

Specification of Letters Patent. Patented Oct. 11, 1921.

No Drawing.

Application filed August 18, 1920. Serial No. 404,377.

To all whom it may concern:

Be it known that I, FOSTER MILLIKEN, a citizen of the United States, and a resident of Lawrence, in the county of Nassau and State of New York, have invented a new and Improved Alloy, of which the following is a full, clear, and exact description.

The object of the invention is to provide a new and improved alloy capable of being rolled, drawn, forged or worked in other ways while being cold, to form rods, plates, sheets, wires, tubing and the like.

An alloy made from the following metals in substantially the following proportions, 15 namely,

|                  | Per cent. |
|------------------|-----------|
| Copper           | 60 to 70  |
| Zinc             | 19 to 24  |
| Nickel           | 9 to 12   |
| Iron             | 1 to 2½   |
| Manganese copper | 1         |

The four ingredients, namely, the copper, nickel, zinc and iron, are melted together to form an alloy and when this alloy is in a molten condition, 1 per cent. of manganese copper is added. The manganese copper used is approximately 28 per cent. manganese and 72 per cent. copper. The manganese deoxidizes the other ingredients and 30 acts as a scavenger and purifier. The bulk of the manganese is converted into manganese oxids and in this condition passes off into the slag. A trace of manganese remains in the alloy and this trace forms an important factor in the physical structure of the alloy. The copper of the manganese copper associates with the copper of the alloy.

The alloy is adapted for cold rolling and 40 working and has the additional advantage of being acid resisting. The manganese in the alloy tends to toughen the same.

Tests of the new alloy have produced the following results: When the metal is rolled and cold drawn to what is known as 10 numbers hard it develops an ultimate tensile strength of 134,500 pounds per square inch; drawn to 11 numbers hard it develops 143,000 pounds per square inch; and drawn 50 to 12 numbers hard it develops a tensile

strength of 163,200 pounds per square inch and a reduction in area (in this last case) of 17 per cent.

It is understood that the tensile strength of the alloy ranges from 45,000 to 183,000 pounds per square inch as the hardness varies from dead soft to say 16 numbers hard, but the above-mentioned numbers are for the alloys most used in commerce.

The alloy is, as previously stated, acid resisting and the following acids, bases, salts and organic compounds are successfully resisted by the alloy:

| Acids.        | 65         |
|---------------|------------|
| Citric.       | Oelic.     |
| Hydrofluoric. | Sulfuric.  |
| Oxalic.       | Sulfurous. |

| Bases.        | 70              |
|---------------|-----------------|
| Caustic soda. | Caustic potash. |

| Salts.            |                   |
|-------------------|-------------------|
| Aluminum sulfate. | Calcium chlorid.  |
| Ammonium citrate. | Calcium sulfate.  |
| Ammonium sulfate. | Sodium phosphate. |

| Organic compounds. |             |
|--------------------|-------------|
| Acetone.           | Chloroform. |
| Benzol.            | Ether.      |

This alloy differs from the one described in the Letters Patent of the United States, No. 1,314,417, granted to me on August 26, 1919, in that it has a high percentage of copper, a low percentage of zinc, and but a trace of manganese.

Having thus described my invention, I claim as new and desire to secure by Letters Patent:

An alloy consisting of the following ingredients in substantially the following proportions: copper, 60 to 70 per cent.; zinc, 19 to 24 per cent.; nickel, 9 to 12 per cent.; iron, 1 to 2½ per cent.; and a trace of manganese and having a tensile strength from 45,000 to 183,000 pounds per square inch as the hardness varies from dead soft to 16 numbers hard.

FOSTER MILLIKEN.